

Mar. 3, 1925.

1,528,205

W. E. GREENAWALT

METALLURGICAL PROCESS

Original Filed March 19, 1915



INVENTOR.

William E. Greenawalt

## UNITED STATES PATENT OFFICE.

WILLIAM E. GREENAWALT, OF DENVER, COLORADO.

## METALLURGICAL PROCESS.

Continuation of application Serial No. 15,583, filed March 19, 1915. This application filed July 22, 1921. Serial No. 486,904. Renewed August 28, 1923.

To all whom it may concern:

Be it known that I, WILLIAM E. GREENAWALT, a citizen of the United States, residing in the city and county of Denver and State of Colorado, have invented certain new and useful Improvements in Metallurgical Processes, of which the following is a specification.

The invention will be described more particularly in reference to the treatment of copper ores, altho it is applicable to other metals. It will be described more particularly in reference to sulphate solutions, altho it is also applicable to chloride and other solutions.

The subject matter of this application is similar to that of my co-pending applications, Serial No. 15,583, filed March 19, 1915; Serial No. 228,952, filed April 16, 1918; and Serial No. 239,255, filed June 10, 1918, or Patents No. 1,340,826, No. 1,480,059; and No. 1,357,495, respectively.

In the extraction of copper from its ores with dilute acid solutions iron is inevitably dissolved with the copper. In the electrolytic deposition of the copper from leach solutions containing iron, ferrous iron is not particularly harmful; it may be decidedly beneficial. Ferric iron is very detrimental; it attacks the deposited copper and causes a loss of efficiency practically in proportion to the ferric iron in the electrolyte. On the other hand, ferric salt has been largely used, and frequently suggested, in the extraction of copper from its ores. It makes a fairly efficient solvent. One of the objections to its use has been the difficulty and expense of its production and regeneration. It acts beneficially in the extraction of the copper from its ores. It acts harmfully in the precipitation of the copper from its solutions. So far as I know it is, and has been, the custom, without exception, in the electrolytic deposition of copper from leach solutions to maintain the ferric iron in the electrolyte at a certain low standard by diverting, or discarding, a portion of the solution, and after precipitating the copper with metallic iron, wasting the diverted solution. It is one of the objects of this process to turn this diverted solution, presumably high in iron, to a profitable account.

In the present process the object is to carry a fairly high iron content in the electrolyte in the deposition of the copper, and maintain the iron reduced, preferably by means of copper sulphide. It is preferred to carry, say, from 2.0% to 5.0% iron in the electrolyte, in the deposition of the copper, and regulate its flow thru the cells in such a way, that while the iron content may be high, only a comparatively small portion, say, from 0.1% to 0.25% will be oxidized to the ferric condition. This may be done by alternately passing the electrolyte thru a number of cells in multiple, and thru reducing units, at such a rate that the solution issuing from the reducers will be practically completely reduced, and the solution issuing from the cells will not exceed 0.25% ferric iron. Ultimately, of course, the iron will accumulate in such amounts in the electrolyte that elimination of part of it becomes desirable, but instead of discarding the solution heavily charged with iron salts by precipitating its copper content with metallic iron and then wasting the solution, I use both the precipitate and the solution to advantage, as I will now describe.

Most leachable ores contain some sulphides as well as oxides. These sulphides, especially in disseminated deposits, are usually in the form of chalcocite and chalcopyrite. Copper in its oxide (including carbonate) combinations is readily soluble in dilute acids, but the sulphides remain practically unaffected. The result is, that the extraction, under the conditions of ordinary dilute acid leaching, is low and unsatisfactory, and does not represent the ultimate possibilities of the process. While the copper in its sulphide combinations is practically unaffected by sulphuric acid, it is readily made soluble in a dilute acid solution of ferric salts, and a very high extraction of the copper is obtainable with an acid solution of ferric salts, from both its oxide and sulphide combinations. To attempt the regeneration of the ferric salts during the electrodeposition of the copper, to a useful degree, is difficult, if not impractical. So far it has proved impractical. The efficient electrolytic deposition of the copper, and the efficient regeneration and accumulation of large

quantities of ferric salts for leaching, are diametrically opposed. This was the idea in the Siemens-Halske process, and it can readily be seen why the process was unsuccessful.

In the present process it is not intended to waste the solution high in iron, but rather to conserve it, and turn it to useful account. When the electrolyte becomes too heavily charged with iron for effective use, a portion is diverted, after the copper electrolysis, to another set of cells, in which the solution high in iron is electrolyzed under oxidizing conditions, and then the acid ferric salt solution is applied to the ore as a wash and to extract the copper from the ore in its sulphide combinations. The copper so extracted is preferably precipitated with hydrogen sulphide, and the copper sulphide so produced is then used to reduce the ferric salts in the copper electrolyte, while an equivalent of copper goes into solution as the sulphate, which, in turn, is electrolyzed in the regular electrolyte to deposit the pure electrolytic metal with the simultaneous regeneration of an equivalent of acid.

The process will now be described more in detail, reference being had to the accompanying drawing, which represents a flow sheet, or diagrammatic sketch, of the preferred method of carrying it out. The ore, suitably crushed, is charged into the leaching vats No. 1 and No. 2. The ore in vat No. 1 is supposed to be a fresh charge, and that in No. 2 is supposed to have been treated with the regular, standard, or primary leaching solution, but still containing some extractable copper in its sulphide combinations, and possibly also in some other combinations not easily extracted by the primary solution.

The primary solution may be considered as being a dilute acid solution containing relatively small amounts of ferric salts. This solution is applied to the fresh ore, as in vat No. 1. The copper solution, issuing from the leaching vat No. 1 and containing also considerable iron, mostly in the ferrous condition, flows into the copper depositing cells No. 1, which are preferably arranged in multiple, and the rate of flow thru the cells is regulated in such a way that only from 0.10% to 0.25% of the iron is oxidized to the ferric condition. The solution or electrolyte, on issuing from the copper cells No. 1 passes into the first reducing unit No. 1, where the ferric iron produced by the deposition of the copper in the first group of copper deposition cells, is reduced to the ferrous condition, preferably by the use of copper sulphide precipitated from the lean and foul solutions produced in another step of the process. The reducing unit will ordinarily consist of an agitator in which the ferric iron is brought in intimate contact

with the precipitated copper sulphide, a separator in which the copper sulphide precipitate is separated from the reduced solution, and a pump to return the settled sulphide sludge from the separator to the agitator. The reduction may be accomplished in a few minutes, especially if the solution is heated. The clear overflowing solution from the separator flows into the next set of copper depositing cells No. 2, where more copper is deposited and more ferrous iron oxidizing to the ferric condition, but this ferric iron, on account of the regulated rate of flow of the electrolyte, should not exceed 0.25%. On issuing from the copper depositing cells No. 2, the electrolyte flows into the reducing unit No. 2, and from the second reducing unit to the third set of copper depositing cells No. 3, and this is continued until the electrolyte is sufficiently impoverished in copper and regenerated in acid, after which it is again returned to the ore to pass thru another cycle. The leaching of the ore in vat No. 1 is continued until the oxidized, or easily extractable, copper is brought into solution and removed; vat No. 1, will then be in the condition of vat No. 2. It is desirable to maintain the ferric iron at not to exceed 0.25% on issuing from each set of deposition cells, and to reduce this amount of ferric iron quickly and as completely as possible in the successive reducing units. There will, of course, be no need of reducing the ferric iron in the last set of depositing cells, and hence a small amount of ferric iron will inevitably be in the primary leaching solution, and may be beneficial in the solution.

Manifestly, if this cycle of solution and deposition is continued indefinitely the iron in the primary solution, or electrolyte, will accumulate in undesirable amounts, even tho the iron content may be maintained high. When it is desired to eliminate some of the iron, or perhaps, to maintain the iron in the primary solution at a certain maximum, a small portion of the primary solution is diverted to form a secondary solution with which to extract the remainder of the copper in the ore after the application of the primary solution. This secondary solution is presumably high in iron. It is treated, preferably by electrolysis, to convert the iron in the ferric condition. This secondary solution then becomes an active solvent of the copper, as in vat No. 2, in its sulphide combinations, and other combinations not readily soluble in dilute acid solutions.

This secondary leaching circuit will now be described. The regenerated ferric salt solution is applied to the leaching vat No. 2, where it acts on the copper remaining after the application of the primary solution. On issuing from the vat it will be rather low in copper and contain most of the iron in the

ferrous condition, altho some of the iron will still be in the ferric state. In order to make all the chemical reactions more positive, it is desirable to heat the solutions. It passes thru the heater in a regulated stream into the  $\text{SO}_2$  reduction chamber where the excess ferric salts is reduced to the ferrous condition with the simultaneous regeneration of an equivalent of acid. The secondary solution, now having the salts of the variable valent elements reduced to their lowest valency, is flowed into the  $\text{H}_2\text{S}$  precipitator, where the copper is easily and completely precipitated from the reduced solution as the sulphide, with the simultaneous regeneration of more acid. The regenerated acid solution now containing ferrous iron in solution and the precipitated copper sulphide in suspension, is flowed into the copper sulphide separator, where the copper sulphide settles to the bottom and the clear overflowing solution passes on to the oxidizing cells in which the reduced acid solution is electrolyzed under oxidizing conditions, to convert the ferrous salts into the ferric salts. The oxidizing action of the electrolysis is improved by agitation; it also assists in the depolarization, reduces the E. M. F. required in the electrolysis, and materially prolongs the life of the anodes. Compressed air for agitation may be introduced into the various cells as desired. Air also assists directly in the oxidizing action, but not energetically. If it is desired to use a more energetic oxidizing agent than air in the conversion of the ferrous salts to ferric salts, in the electrolysis, manganese dioxide may be used. Manganese dioxide is an effective oxidizer of the ferrous salts, and may also act as a depolarizer. If it is to be used as an oxidizing agent, it is preferably ground fine and introduced with the solutions into the oxidizing cells. The air agitation prevents it from settling in the cells, and it flows out with the ferric solutions, into the separator, where it is separated from the regenerated ferric solution and again returned to the cells. The clear overflowing acid solution, now containing much of the iron in the ferric condition, is returned to the ore in vat No. 2, and the cycle repeated until the copper is sufficiently extracted. The ore is then washed, and necessarily some of the solvent must be wasted as in all leaching processes, and the portion of the solvent which is necessarily wasted will just about keep the secondary solvent at a desired standard of iron. If it is desired to have a high iron content in the secondary solution, the ferrous sulphate from the hydrogen sulphide generator may be added to the solution. The hydrogen sulphide may be generated in a number of ways, but for the purpose of this process it is preferred to generate it by the reaction between iron sulphide and dilute sulphuric acid.

Within certain limits, the higher the iron in the secondary solution the more effective will be the oxidation and consequent depolarization. It is not necessary to oxidize all of the ferrous iron. It is preferable not to do so. Suppose the secondary leaching solution contains 5.0% total iron. If 2.0% to 3.0% of this is oxidized to the ferric condition it will give a very active solvent for the copper in the ore in its sulphide combinations; while the remaining 3.0% to 2.0% ferrous iron still leaves enough of the iron unoxidized to effectively act as a depolarizer, to maintain a low E. M. F., and to greatly prolong the life of the anodes.

While small amounts of copper in the secondary solution during oxidizing electrolysis is not harmful, it is preferred to precipitate the copper chemically and then electrolyze the secondary solution under highly oxidizing conditions. The copper deposited in the oxidizing cells would result in an impure metal, a very poor efficiency at the cathode, and a reduced efficiency at the anode. The copper sulphide precipitate, from the impure secondary solution, is quite pure and can be used effectively in the reduction of the ferric salts in the primary solution, and can in this way ultimately all be converted into the pure electrolytic metal while performing the very important function of reducing the ferric salts and generation of acid.

It is preferred to heat the solution, especially in the secondary circuit, for the reason that sulphur dioxide reduction, as well as hydrogen sulphide precipitation, takes place more effectively in heated than in cold solutions, and the precipitate settles more rapidly, and in the oxidizing electrolysis, oxidation is more readily effected and the depolarization may be made practically complete under the conditions of this process.

While sulphur dioxide is preferred as a reducing agent, preparatory to precipitation with hydrogen sulphide, it is not essential. Hydrogen sulphide will reduce the ferric salts more effectively than sulphur dioxide, but there is more acid regenerated by the use of sulphur dioxide. There is no sulphur precipitated with sulphur dioxide reduction, and the copper sulphide precipitate with hydrogen sulphide is of a higher grade when the reduction is made with sulphur dioxide. Then, too, sulphur dioxide is a waste gas in most copper metallurgical works, and is rarely, if ever, as expensive as hydrogen sulphide.

It is desirable, in this process, to have some acid in the secondary solution. The acid materially assists in the electrolytic oxidation of the ferrous salts, and greatly improves the action of the ferric salts in the extraction of the copper from the ore, especially if the solution is heated.

It is not intended to draw a sharp line between the application of primary and secondary leaching solutions to the ore. As soon as the primary leaching is finished, it is preferred to follow it up immediately with the secondary solution, and the operator will soon learn when to switch the issuing copper solution from the primary to the secondary circuit.

10 A close separation need not be made between the copper sulphide precipitate and the reduced regenerated acid secondary solution. It is preferred to draw the copper sulphide precipitate from the bottom of the 15 separator as a thickened sludge and flow it into the agitators of the primary circuit.

The process may be carried out in any convenient apparatus. The leaching apparatus and copper deposition cells may be of 20 any standard design. For the reducing units, Dorr agitators and Dorr thickeners, or separators, are preferred. These separators are also preferred for separating the copper sulphide precipitate in the secondary 25 solution. For the sulphur dioxide reduction and hydrogen sulphide precipitation an apparatus such as that shown in my co-pending application Serial No. 16,962, filed March 25, 1915, (Patent No. 1,347,089) is 30 preferred, and for the oxidizing electrolysis an apparatus such as that shown in my co-pending applications Serial No. 145,884, filed February 1, 1917, (Patent No. 1,347,088) and Serial No. 231,534, filed April 29, 1918, 35 (Patent No. 1,365,032) is preferred.

It is desirable to have a fairly violent agitation in the oxidizing cells, and this is possible when there is no copper to be deposited. In the presence of ferric salts, 40 violent agitation, while it materially assists in the depolarization, also assists in redissolving the copper, if it is attempted to deposit copper while regenerating ferric salts.

The sulphide precipitate, resulting from 45 the precipitation of the copper in the secondary solution, with hydrogen sulphide, may be separated from the reduced and regenerated acid solution by flotation instead of by gravity, in a Dorr thickener. The sulphide 50 precipitate is easily floated, and sometimes this method may be preferred. If preferred, the CuS separator may be represented by any of the well known flotation machines.

Lead, ferrosilicon, or magnetite anodes 55 will ordinarily be used to deposit the copper from the primary solution. Carbon anodes will ordinarily be used in electrolyzing the secondary solution: there will be no difficulty in maintaining good depolarization of the 60 carbon anodes in a sulphate solution high in ferrous iron, under the conditions of agitation and elevated temperature of the electrolyte as contemplated in the operation of this step of the process.

65 The process has been described in connec-

tion with sulphate solutions; it is equally applicable with chloride solutions.

I claim:

1. A process of extracting copper from its ores, which consists in first treating the ore 70 with an acid solution relatively low in ferric iron to extract a portion of the copper, and then treating the ore with an acid solution relatively high in ferric iron to extract the remainder of the copper, and separately precipitating the copper from both solutions. 75

2. A process of extracting copper from its ores, which consists in first treating the ore with an acid solution relatively low in ferric iron to extract a portion of the copper, 80 and then treating the ore with an acid solution relatively high in ferric iron to extract the remainder of the copper, precipitating the copper from the first solution electrolytically, and precipitating the copper from 85 the second solution chemically.

3. A process of extracting copper from its ores which consists, in first treating the ore with an acid solution to extract a portion of 90 the copper, and then treating the ore with an acid solution containing ferric iron to extract the remainder of the copper, precipitating the copper in the first solution electrolytically, precipitating the copper in the second solution chemically, and treating the 95 first solution with the chemically precipitated copper from the second solution.

4. A process of extracting copper from its ores containing the copper in its oxide and sulphide combinations which consists, in first 100 treating the ore with an acid solution to extract the copper in its oxide combinations, then treating the ore with a solution containing ferric iron to extract the copper in its sulphide combinations, and separately 105 treating the copper from both solutions.

5. A process of extracting copper from its ores which consists, in treating the ore with a primary acid solution to extract a portion 110 of the copper, then treating the ore with a secondary solution containing ferric iron to extract the remainder of the copper, precipitating the copper from both solutions separately, and separately returning both solutions to the ore. 115

6. A process of extracting copper from its ores which consists, in treating the ore with a primary acid solution to extract a portion of the copper, then treating the ore with a secondary solution containing ferric iron to 120 extract the remainder of the copper, electrolytically precipitating the copper from the primary solution, and chemically precipitating the copper from the secondary solution, and separately returning both solutions to the ore. 125

7. A process of extracting copper from its ores which consists, in treating the ore with a primary acid solution to extract a portion 130 of the copper, then treating the ore with a

- secondary solution containing ferric iron to extract the remainder of the copper, electrolytically precipitating the copper from the primary solution, chemically precipitating the copper from the secondary solution, separately returning both solutions to the ore, and treating the primary solution with the precipitate obtained from the secondary solution to reduce the salts of the variable 10 valent elements in the primary solution from a higher to a lower valency.
8. A process of extracting copper from its ores which consists, in treating the ore with a primary acid solution to extract a portion 15 of the copper, then treating the ore with a secondary solution containing ferric iron to extract the remainder of the copper, electrolytically precipitating the copper from the primary solution, chemically precipitating the copper from the secondary solution, electrolyzing the secondary solution to convert the ferrous iron to the ferric condition, and returning both solutions separately to the ore.
- 20 9. A process of extracting copper from its ores which consists, in treating the ore with a primary acid solution to extract a portion of the copper, then treating the ore with a secondary acid solution containing ferric 25 iron to extract the remainder of the copper, electrolytically precipitating the copper from the primary solution; chemically precipitating the copper from the secondary solution as the sulphide, electrolyzing the 30 secondary solution to convert the ferrous iron in the solution to the ferric condition, separately returning both the primary and 35 secondary solutions to the ore, and treating the primary solution during the electrolytic precipitation with the sulphide precipitate 40 from the secondary solution.
10. A process of extracting copper from its ores which consists, in treating the ore with a primary acid solution containing iron 45 salts to extract a portion of the copper, electrolyzing the resulting solution to deposit the copper, diverting enough of the primary solution as it becomes undesirably charged with iron to form a secondary solution, electrolyzing the secondary solution to convert the ferrous iron to the ferric condition, and then applying the regenerated ferric 50 solution to the ore to extract the remainder of the copper.
- 55 11. A process of extracting copper from its ores which consists, in treating the ore with an acid solution to extract a portion of the copper, electrolyzing the resulting copper solution containing salts of iron to 60 deposit the copper and regenerate acid in such a way as to prevent the accumulation of ferric iron in the electrolyte, and then electrolyzing the solution in such a way as to promote the formation and accumulation of the ferric iron, and then applying 65
- the regenerated ferric iron solution to the ore to dissolve the remainder of the copper.
12. A process of treating ores of metals which consists, in treating the ore with an acid solution to extract a portion of the 70 metals, electrolyzing the resulting metal solution containing salts of iron to deposit the metals in such a way as to retard the formation and accumulation of ferric iron in the electrolyte, and then electrolyzing the 75 solution in such a way as to promote the formation and accumulation of the ferric iron, and then applying the regenerated ferric salt solution to the ore to extract the remainder of the metals.
- 80 13. A process of extracting copper from its ores which consists, in treating the ore with an acid solution to dissolve the copper, electrolyzing the resulting copper solution containing salts of iron to deposit the copper and subjecting the electrolyte to the action of a reducing agent, and then after the electrolyte is sufficiently impoverished in copper and regenerated in acid electrolyzing 85 it again and subjecting it to the action of an oxidizing agent.
14. A process of extracting copper from its ores which consists, in treating the ore with a primary acid solution to extract a portion of the copper, electrolyzing the solution to deposit the copper, diverting enough of the primary solution to form a secondary solution and in such a way as to prevent an undesirable excess of iron salts 95 in the primary solution, treating the secondary solution to convert the iron from the ferrous to the ferric condition, applying the secondary ferric solution to the ore to extract the remainder of the copper, and chemically precipitating the copper in the 100 secondary solution.
15. A process of extracting copper from its ores which consists in part of maintaining separate a primary and a secondary solution circuits, and passing the excess of iron 110 salts in the primary circuit to the secondary circuit, electrolyzing the iron salt solution in the secondary circuit under oxidizing conditions to convert the iron into the ferric condition, and then applying the ferric iron 115 solution so obtained to extract copper from the ore in its sulphide combinations.
16. In the treatment of copper ores in which a portion of the copper is soluble in dilute acid and another portion soluble in 120 a solution of ferric salts, the process comprising subjecting the ore successively to the action of a primary solvent relatively low in ferric iron to extract the readily soluble copper and then to the action of a solvent relatively high in ferric iron to extract the copper not readily soluble in the 125 primary solution.
17. A process of extracting copper from its ores which consists in part of subjecting 130

- the ore successively to the action of a primary solvent relatively low in ferric iron and to the action of a solvent relatively high in ferric iron, precipitating the copper from 5 both solvents separately, and separately returning the solvents to the ore.
18. A process of extracting copper from its ores which consists in treating the ore with a solvent for the copper, electrolyzing 10 the solution containing salts of iron to deposit the copper under conditions to retard the formation and accumulation of ferric iron, and then when the solution becomes undesirably charged with iron salts 15 diverting a portion of the solution and electrolyzing the diverted portion to promote the formation and accumulation of ferric iron, and then applying the resulting ferric salt solution to the ore.
19. A metallurgical process which consists in treating ores of metals with a solvent for the metals, electrolyzing the resulting metal solution to deposit the dissolved metal values and regenerate the solvent, repeating 20 the cycle until the solution becomes sufficiently charged with impurities, then diverting a portion of the solution and chemically precipitating the remaining metal values from the diverted foul solution, and 25 then applying the barren foul solution to the ore.
20. A metallurgical process which consists in treating ores of metals with a solvent for the metals, electrolyzing the resulting 30 metal solution to deposit the dissolved metal values and regenerate the solvent, repeating the cycle until the solution becomes sufficiently charged with impurities, then diverting a portion of the solution and chemically precipitating the remaining metal values from the diverted foul solution, and 35 then applying the electrolyzed barren solution to the ore.
21. A metallurgical process by which ores of copper are treated with a primary acid solution to extract a portion of the copper and a secondary solution high in iron salts to extract the remainder of the copper, the 40 steps which consist in chemically precipitating the copper from the secondary solution, separating the chemical precipitate from the resulting solution, and then treating the primary solution with the chemical 45 precipitate from the secondary solution.
22. A metallurgical process by which ores of copper are treated with a primary solution to extract a portion of the copper and a secondary solution containing salts of iron 50 to extract the remainder of the copper, the steps comprising electrolytically precipitating the copper from the primary solution, chemically precipitating the copper from the 55 secondary solution, separating the resulting chemical precipitate from the secondary
- solution, electrolyzing the barren secondary solution, and returning the electrolyzed barren solution containing ferric iron to the ore.
23. A process of treating ores of copper 70 comprising leaching the ore with a dilute acid solution to extract a portion of the copper, alternately electrolyzing and reducing the resulting copper solution containing salts of iron to deposit the copper and regenerate acid until the solution is sufficiently depleted in copper and regenerated in acid, then returning a portion of the regenerated acid solution to the ore and chemically precipitating the remaining copper from another portion, electrolyzing the resulting solution from which the copper has been chemically precipitated to regenerate ferric salts, and then returning the resulting ferric 75 salt solution to the ore to extract another 80 portion of the copper.
24. A process of treating ores of copper, comprising leaching the ore with an acid solution containing salts of iron to extract a portion of the copper, precipitating a portion 85 of the copper electrolytically with the simultaneous regeneration of acid, then precipitating a portion of the copper chemically with the regeneration of more acid, then treating the solution from which the copper has been chemically precipitated to convert the ferrous salts into the ferric condition, and then returning the regenerated ferric salt solution to the ore.
25. A process of treating copper ores, 90 comprising leaching the ore with an acid solution containing salts of iron to extract a portion of the copper, precipitating a portion of the copper from the solution electrolytically with the simultaneous regeneration of acid, precipitating a portion of the copper chemically with the simultaneous regeneration of more acid, then electrolyzing the resulting solution depleted in copper 95 and agitating the electrolyte with air to convert the ferrous iron in the solution into the ferric condition, and then returning the regenerated acid ferric salt solution to the ore to dissolve more copper.
26. A process of treating copper ores, 100 comprising leaching the ore with a solvent containing salts of iron to extract a portion of the copper, chemically precipitating the copper from the solution so that the solution will be practically free from copper, 105 then electrolyzing the resulting solution to convert the ferrous iron into the ferric condition and agitating the electrolyte during electrolysis, and then returning the regenerated ferric salt solution to the ore to extract 110 more copper.
27. A process of treating ores of metals comprising, leaching the ore with a primary solution relatively low in ferric salts to extract a portion of the metals, then leaching 115

the ore with a secondary solution relatively high in ferric salts to extract the remaining metals, precipitating the metals from the secondary solution, applying the precipitate from the secondary solution to the primary solution, and then electrolyzing the primary solution to deposit the metals.

28. A process comprising, treating ores of metals with a primary solution relatively low in ferric salts to extract a portion of the metals, then treating the ore with a solution relatively high in ferric salts to extract the remaining metals, precipitating the metals from the secondary solution and returning the secondary solution to the ore, applying the precipitate from the secondary solution to the primary solution, then electrolyzing the primary solution to deposit the metals and regenerate the solvent and returning the regenerated primary solution to the ore.

29. In the treatment of copper ores in which a portion of the copper is soluble in dilute acid and another portion soluble in a ferric salt solution, the process comprising subjecting the ore successively to the action of a primary solvent relatively low in ferric iron to extract the readily soluble copper and then to the action of a secondary solvent relatively high in ferric iron to extract the copper not readily soluble in the primary solution, electrolytically precipitating the copper from the primary solution, chemically precipitating the copper from the secondary solution, then electrolyzing the secondary solution with carbon anodes, and returning the electrolyzed solution to the ore.

30. In the treatment of copper ores in which a portion of the copper is soluble in

dilute acid and another portion soluble in a ferric salt solution, the process comprising subjecting the ore successively to the action of a primary solvent relatively low in ferric iron to extract the readily soluble copper and then to the action of a secondary solvent relatively high in ferric iron to extract the copper not readily soluble in the primary solution, precipitating the copper from the primary solution by electrolysis, precipitating the copper from the secondary solution with hydrogen sulphide generated from ferrous sulphide and acid, adding the resulting ferrous salt from the generation of hydrogen sulphide to the secondary solution, treating the secondary solution to convert the ferrous iron to the ferric iron, and returning the solution to the ore.

31. In the treatment of copper ores in which a portion of the copper is soluble in dilute acid and another portion soluble in a ferric salt solution, the process comprising subjecting the ore successively to the action of a primary solution relatively low in ferric iron to extract the readily soluble copper and then to the action of a secondary solution relatively high in ferric iron to extract the copper not readily soluble in the primary solution, precipitating the copper from the primary solution separately from the secondary solution, chemically precipitating the copper from the secondary solution, then electrolyzing the secondary solution in the presence of a substance other than air which is capable of promoting the production of ferric salts, and returning the electrolyzed solution to the ore.

WILLIAM E. GREENAWALT.